

## UNITED STATES PATENT OFFICE

2,033,927

PROCESS OF MAKING A METAL ARTICLE OF  
PRECISE DIMENSIONS AND THE ARTICLE  
PRODUCED THEREBY

Henry A. De Fries, Cleveland, Ohio, assignor, by  
mesne assignments, to The Nitralloy Corpora-  
tion, a corporation of Delaware

No Drawing. Continuation of application Serial  
No. 273,432, April 27, 1928. This application  
February 20, 1932, Serial No. 594,389

## 12 Claims. (Cl. 148—16)

5 My invention relates to devices which are generally classified as tools and comprising for instance, gauges, drawing dies, forming dies, boring bars, mandrels, burnishers and the like, all of which are required to be made to exact dimensions and precise forms and therefore may be classified generally as instruments of precision.

10 Some instruments of this character, such as gauges for example, are not subjected to high pressure or other severe stresses, whereas others, such as forming dies, must sustain considerable loads. All such instruments, however, require a hard, wear-resisting surface, and it is highly desirable that such surface be of a stable, non-corrosive character.

15 In the manufacture of such devices it has long been the practice to make them of hardened or case carburized steels. With the ordinary processes the maximum degree of hardness which can be obtained does not exceed 750 Brinell, and it is very difficult to prevent deformation and distortion of the pieces due to the quenching operation necessary in the hardening process.

20 It is known that certain steels can be surface hardened by the so-called nitriding process as described in United States Patent No. 1,487,554, issued to Adolf Fry on March 18, 1924. By this process, I find that machined and heat treated pieces can be hardened at such low temperatures as to retain the physical properties imparted to 25 the cores thereof prior to nitriding, and if proper precautions are taken, may be done without any distortion or deformation. Furthermore, the hardness which can be imparted to the surface ranges between 900 and 1100 Brinell.

25 The steels most suitable for this process are the so-called "Nitralloy" or aluminum bearing steels as described in another United States Patent No. 1,649,398 issued to Fry on November 15, 1927. In using these steels, however, I have found that the best results are obtained by dividing them into two series, to wit: First, an aluminum bearing steel of medium carbon content for those instruments which do not require a core hardness of more than 300 Brinell; and second, an aluminum bearing 30 steel of higher carbon content for those instruments which require a core hardness in excess of 300 Brinell.

35 In the first series, a carbon content of from 0.15% to 0.50% is recommended, while for the second series, steels containing from 0.50% to 2.0% carbon (the other alloying elements being in proportion) are recommended.

40 For example, where the instrument does not require a core hardness in excess of 300 Brinell,

a steel of about the following composition will prove satisfactory:

|              | Per cent  |
|--------------|-----------|
| Carbon       | 0.25-0.35 |
| Chromium     | 1.50-1.75 |
| Manganese    | 0.50-0.60 |
| Silicon      | 0.20-0.30 |
| Molybdenum   | 0.15-0.25 |
| Aluminum     | 1.00-1.25 |
| Balance iron | 10        |

45 Such a steel annealed will give about 170 Brinell, and when quenched in oil from 1650 degrees F. and tempered at about 1050 degrees F. will attain a Brinell hardness of about 300.

50 When an instrument having a greater core hardness is required, a steel of the following composition will be found satisfactory:

|              | Per cent  |
|--------------|-----------|
| Carbon       | 0.70-0.80 |
| Chromium     | 1.75-2.00 |
| Manganese    | 0.50-0.60 |
| Silicon      | 0.20-0.30 |
| Molybdenum   | 0.25-0.35 |
| Aluminum     | 1.50-1.75 |
| Balance iron | 25        |

55 Such a steel annealed will give about 200 Brinell and when quenched in oil from 1600 degrees F. and tempered at 1050 degrees F. will attain a Brinell hardness of about 480. This same steel, if heated to 1600-1700 degrees F. and air cooled, will attain a Brinell hardness of 600. In any case the hardness in either series will vary somewhat with different tempering heats.

60 In the manufacture of instruments by my process, it should always be borne in mind that nitriding subjects the steel to prolonged heating at about 900 degrees F., and for this reason any tempering or core hardening which is done prior to nitriding should be done at a temperature in excess of 900 degrees F. Furthermore, it is obvious that no case, however hard in itself, is ever stronger than the core which supports it, and that the case itself on account of its extreme hardness must be somewhat less elastic than the steel before hardening. Therefore, it is quite essential that a supporting core of sufficient hardness should be provided to prevent the case from being stressed to the cracking point. Hence it is important that steel with the proper carbon content to provide the requisite hardness be selected.

65 A plug gauge, for example, sustains no load, and, therefore, low carbon steel annealed and nitrided can be used. On the other hand, prac-

tice has shown that a wire drawing die requires a core hardness of from 400 to 500 Brinell in order to withstand the pressure developed when the wire is drawn through the opening therein.

5 After having selected a steel in which the required physical properties of the core may be developed by suitable heat treatment, a working surface may be applied thereto which will be extremely hard, extremely resistant to wear, and absolutely rustless in so far as atmospheric, fresh and salt water corrosion is concerned, thereby combining all these desirable requisites in the same unit.

10 In the manufacture of instruments of precision which require only annealing, I proceed as follows: The part is first rough formed by machining or otherwise from steel containing elements adapting it to be nitrided and which preliminary to the rough forming or machining operation 15 preferably has been annealed. Where the instrument is of simple section it will not be necessary to reheat the roughly formed part, but where a complicated section is involved it should be thoroughly reheated to a temperature sufficient 20 to relieve any internal strains developed in forging or machining. After rough forming of a simple section or after the rough forming and reheating of a more complicated section, it is finished by machining and grinding to the precise 25 dimensions required, and is then nitrided to harden the surface.

30 During the nitriding, while there is no distortion or deformation, there is a very slight growth due to the absorption of nitrogen. This growth is only about 0.0003 to 0.0010 inch depending upon the duration of the treatment. Where this growth exceeds the tolerance allowed, the instrument may, thereafter, be reduced to exact size by a slight lapping operation. Otherwise, allowance 35 may be made for this slight growth in the fine machining and grinding, and the lapping omitted.

35 Where the instrument requires heat treatment for hardening the core, I proceed as follows: The device is first rough formed by machining or otherwise from steel containing elements adapting it to be nitrided and which preferably has been previously brought to the annealed state. The rough formed part is then heat treated 40 for the purpose of developing the required physical properties by subjecting to a hardening heat treatment followed by tempering. If the section is of simple character it need not be reheated after the rough forming operation and before subsequent working or heat treatment operations, but, otherwise, it should be reheated to relieve any internal strains set up during the rough forming. After reheating to relieve internal strains followed by heat treatment to develop 45 the desired core hardness, or, if a simple section, after rough machining and heat treatment to develop the required physical properties, the instrument is finish-ground to the exact required dimensions. It is then nitrided, and may thereafter be lapped if the growth during the nitriding exceeds the tolerance allowed and no allowance for the growth has been made in the finish grinding. The reheating treatment to relieve internal strains set up during machining or 50 other working operations may constitute a full anneal or a normalizing treatment when it precedes the heat treatment for developing core hardness. If it occurs after the hardening heat treatment, then the temperature in such reheating treatment should not be carried above the

5 drawing temperature employed in the hardening heat treatment.

Sometimes a thin film of oxide appears on the surface of the nitrided article. If objectionable, this film can be readily removed with fine emery 5 cloth.

From the foregoing it will be apparent that instruments of precision may be made in the manner described to exact desired form and dimensions and without fear of distortion during 10 hardening.

The case produced by a ninety hour nitriding treatment will be about 0.031 inch deep. The outer half is extremely hard, and the case merges gradually into the core without any line of demarcation. For this reason a nitrided instrument 15 cannot suffer from spalling or exfoliation as so frequently occurs in parts poorly carburized.

Growth or distortion greatly in excess of that normally to be expected, as stated above, is an 20 indication that the preliminary forging, machining and reheating operations have not been performed with sufficient care. All strains set up by forging or heavy machining must be relieved by an appropriate drawing or annealing 25 heat treatment, and all scale, resulting from forging or heat treatment, should be removed from surfaces that are to be subsequently nitride hardened.

25 This is a continuation of my application Serial 30 No. 273,432 filed April 27, 1928.

I claim:

1. The process of making a metal article of precise dimensions having an extremely hard, rust and wear-resisting surface which comprises 35 rough forming the article to the approximate dimensions from steel containing elements adapting it to be nitrided, heat treating and tempering the article to provide the necessary core hardness, grinding to precise dimensions; and thereafter 40 nitriding to harden the surface portions.

2. The process of making a metal article of precise dimensions having an extremely hard, rust and wear-resisting surface which comprises 45 rough forming the article to the approximate dimensions from steel containing elements adapting it to be nitrided, heat treating and tempering the article to provide the necessary core hardness, reheating to a temperature sufficiently high to relieve internal strains but below the drawing 50 temperature, grinding to precise dimensions, and thereafter nitriding to harden the surface.

3. The process of making a metal article of precise dimensions having an extremely hard, rust and wear-resisting surface which comprises 55 rough forming the article to the approximate dimensions from steel containing elements adapting it to be nitrided, heat treating and tempering the article to provide the necessary core hardness, grinding to precise finished dimensions, 60 nitriding to harden the surface portions, and thereafter lapping to exact dimensions.

4. The process of making a metal article of precise dimensions having an extremely hard, rust and wear-resisting surface which comprises 65 rough forming the article to approximate dimensions from steel containing elements adapting it to be nitrided, heat treating and tempering the article to provide the necessary core hardness, reheating to a temperature sufficiently high to 70 relieve internal strains but below the drawing temperature, grinding to exact finished dimensions, nitriding, and thereafter lapping to exact finished dimensions.

5. Those steps in the manufacture of a metal 75

article of precise form and dimensions having a nitrided case of extreme hardness and resistance to rust and wear, which comprises heat treating and tempering the article at a temperature above about 900 degrees F. to harden the core, reheat-  
ing to a temperature sufficiently high to relieve 5 internal strains but below the drawing tempera-  
ture, and thereafter nitriding.

6. Those steps in the manufacture of a metal article of precise form and dimensions having a nitrided case of extreme hardness and resistance to rust and wear, which comprise heat treating and tempering the article at a temperature above about 900 degrees F. to harden the core, and 10 thereafter nitriding to harden the surface.

7. The method of nitriding articles made from steel alloys, which comprises heating the articles to a temperature above their upper critical point, quenching the articles, drawing the articles at a 20 temperature below their lower critical point, and then nitriding the articles, the object of said heat treatment being to increase the depth and hardness of the nitrided case to a degree greater than is obtainable when the articles are nitrided without being thus previously heat treated.

8. The method of nitriding articles made from steel alloys, which comprises heating the articles to a temperature of about 1650° F., quenching the articles, drawing the articles at a temperature of about 1050° F., and then nitriding the articles, the object of said treatment being to increase the depth and hardness of the nitrided case to a degree greater than is obtainable when the articles are nitrided without being thus previously heat treated.

35 9. As a new article of manufacture, an instru-

ment of precision having a nitride hardened surface and composed of steel containing carbon from about 0.15% to about 2.0% with aluminum from 0.5% to 2.0%; said instrument being characterized by having its core zone hardened by 5 heat treatment.

10. As a new article of manufacture an instrument of precision required to withstand high pressures and composed of steel having its core zone hardened by heat treatment, and in its marginal layers a rust and wear-resisting nitrided case.

11. An article which in its normal use is subjected to high pressures or shocks in at least a part thereof; said article being composed, at least 15 in those parts which are subjected to such high pressures or shocks, of a steel alloy containing chromium and aluminum and which is susceptible of acquiring such a high hardness in its core portions when subjected to a hardening heat 20 treatment that the Brinell hardness in the core does not decrease below about 300 when said hardened steel alloy is reheated to around 1050° F., said article having its core hardened by heat treatment as aforesaid and having at least the 25 parts thereof which are subjected to such high pressures or shocks surface hardened by nitriding.

12. An article which in its normal use is subjected to high pressures or shocks; said article 30 consisting of a steel alloy containing chromium and aluminum and having a nitride hardened surface and a heat treated core portion, said core portion having a hardness of about 400 or more Brinell.

HENRY A. DE FRIES.

35